

## UNITED STATES PATENT OFFICE.

JUDSON A. DE CEW, OF MOUNT VERNON, NEW YORK, ASSIGNOR TO PROCESS ENGINEERS INC., OF NEW YORK, N. Y.

## METHOD OF SIZING CELLULOSE FIBERS.

No Drawing.

Application filed June 7, 1924. Serial No. 718,657.

*To all whom it may concern:*

Be it known that JUDSON A. DE CEW, a citizen of the United States, residing at Mount Vernon, in the county of Westchester and State of New York, has invented certain new and useful Improvements in Methods of Sizing Cellulose Fibers, of which the following is a specification.

Engine sizing of machine made paper by means of rosin size and sulphate of alumina is carried on in the beating engine or mixer. Sometimes the alum is added before the size and sometimes the size is added to the paper stock before the alum.

15 The size is always coagulated by means of the alum before the beater is discharged.

After the stock leaves the beater, it is passed through a beating or grinding engine, called a jordan, where a violent beating action is given to the mass.

20 The coagulated sizing material is in a very highly dispersed and hydrated condition when it is freshly precipitated but as it passes through the jordan in the presence of excess of sulphate of alumina, the violent beating action has a strong dehydrating action on the alumina and rosin hydrates. Moreover, the sizing material that is precipitated upon the surface of the fibers will 25 be scraped off and left as a filling material between the fibers.

30 The discovery of this fact explains why the sizing from the paper machine is never as efficient as that carried out by means of 35 laboratory tests.

Another disadvantage of the present method of operation is the amount of corrosion that always takes place in the jordan

engine from the presence of sulphate of alumina in the stock. This means rapid 40 wearing down of the knives and constant replacements.

I have discovered that these disadvantages can be avoided by not precipitating the size until the stock has passed through the jordan engine and is ready for the paper machine, and in this way a fresh highly hydrated precipitate is formed which has great covering power and sizing value.

My method of operation is to add the 50 rosin size to the beating engine and coagulate it after it leaves the jordan by bringing an alum solution into contact with the stock in the pipes or machine chest. I may also do all of the sizing in a separate chest after 55 the stock comes from the jordan.

By this method chemical impurities do not injure the sizing to the same extent as they do, when the precipitated size is subjected to dehydration influences.

60 What I claim as my invention is:

1. The method of sizing paper which consists in withholding the precipitation of the rosin until after the beating action of the jordan engine is complete.

65 2. The method of sizing paper which consists in adding the rosin size to the beating engine and co-agulating said size after the paper stock has passed through the jordan.

3. The method of producing with paper 70 pulp an undehydrated precipitate of rosin and alumina which consists in adding the alum to the fibers just before the fibers go to the paper machine.

In testimony whereof I affix my signature.  
JUDSON A. DE CEW.